

## UNITED STATES PATENT OFFICE

2,500,080

INSOLUBILIZATION OF A SOLUBLE AZOIC  
DYESTUFF ON THE FIBER

Robert Lazare Lantz, Paris, France, assignor to  
Societe Anonyme de Matieres Colorantes et  
Produits Chimiques Francolor, Paris, France,  
a corporation of France

No Drawing. Application January 17, 1946, Serial  
No. 641,873. In France February 2, 1945

6 Claims. (Cl. 8—49)

1

This invention relates to a method for the obtention, particularly on the fibres, of water insoluble azoic dyestuffs and to the dyed fibres resulting therefrom.

It has been found that the azoic dyestuffs which possess a secondary amino group in which the hydrogen atom bound with the nitrogen atom is substituted by a sulphonate group have the property of loosing this group when submitted to an acid treatment. If they possess no other solubilizing groups, they thus become insoluble in water. If the initial soluble dyestuff is applied on any kind of fibre it becomes insoluble on the latter in the course of the acid treatment. This discovery leads, therefore, to a new and particularly simple method for preparing insoluble dyestuffs on the fibre. The application of the soluble dyestuff on the fibre may be realized by dyeing, foularding or printing. It may be obtained on vegetable fibres as well as on animal or artificial fibres.

The application on animal fibres or on artificial fibres behaving in a similar manner may be realized like that of an acid dyestuff through dyeing in a bath which should not be too acid if it is desired to avoid a simultaneous developing of the dyestuff. It is possible to add to the bath a reagent, such as borax, an acetate, e. g. sodium acetate or ammonium acetate, soap and the like maintaining the pH between favourable values. In certain cases the developing may be effected simultaneously with the dyeing in order to avoid a complementary operation.

The application through foularding or printing may be obtained by using known methods. The solutions and colours which contain the dyestuff may, besides, contain the various ingredients recommended for similar operations and more particularly solubilizing, or hygroscopic substances or the like. The developing may be effected by any known means capable of reducing the pH of the fibre: steeping in a bath showing the desired acidity at a suitable temperature, passage through an acid atmosphere containing or not containing steam, introduction onto the fibre of a product bringing the fibre to a desired pH through a following treatment such as a steaming process. To this end, salts of volatile bases such as ammonium salts, esters regenerating their acid through hydrolysis or certain salts such as fluorosulphonates, iminodisulphonates and the like may be used.

Azoic dyestuffs which possess a secondary group in which the hydrogen atom bound to nitrogen is substituted by a sulphonate group may

2

be prepared, for instance, according to the method described in our co-pending application No. 641,874, January 17, 1946, now abandoned, entitled "Method for the preparation of diazoic derivatives and azoic dyestuffs derived therefrom," which method consists in coupling with any coupling components the diazoic derivatives obtained by diazotizing an arylene diamine both amino groups of which are substituted by a sulphonate group, one of the said groups furthermore carrying an organic radical. The co-pending application referred to discloses that the sulphonated arylene-diamines used as starting materials may be prepared by the action of sulphonating agents mixed or combined with a tertiary amine on arylene-diamines one of the amino groups of which is a primary group while the other is a secondary group.

As sulphonating agents one may use those which have already been recommended for similar operations, for instance sulphuric anhydride, sulphuric chlorhydrin, chlorosulphonic ester, oleum and pyridinium sulphate. As tertiary amines which may be mixed or combined with the sulphonating agents one can quote pyridin, dimethylaniline and other similar amines. The reaction may be effected in the presence of a solvent or of a diluent.

The coupling is carried out by means of the classical method which consists in dissolving the diazo in the form of a solution or an aqueous paste, in presence of an aqueous solution of the coupling component. According to the nature of said components, the operation takes place in an acid or basic medium. The coupling is carried out at ordinary temperature.

The following are non-limitative examples of realization of the invention, the parts given being parts in weight.

40

*Example 1*

10 parts of wool yarn are introduced into a bath heated to 80° C. and prepared with 300 parts of water, 0.3 part of the dyestuff resulting from the coupling of the diazo-4-phenyl-N-amino-1-benzene-N-sulphonic acid prepared according to the above mentioned co-pending application with (hydroxy-2-naphthoyl-3)amino-benzene, and 0.3 part of ammonium acetate; the temperature is progressively raised so as to reach 95° C. after half an hour. Said temperature is maintained during half an hour whereafter the sample is removed and immersed during a quarter of an hour into a bath of 300 parts of boiling

## 3

water containing 1% of sulphuric acid. The dyeing which was garnet-red before this latter acid treatment turns to purplish-blue. It is then washed with water.

It is also possible to conduct the developing in the first dyeing bath through adding to the same, after the rising of the dyestuff, a quantity of acid sufficient to obtain a slightly acid reaction to Congo red which maintains during the whole operation.

## 4

## Example 2

1 part of loaded or non-loaded silk is dyed in 30 parts of water containing 0.02 part of dye-stuff and 1 g. of soap per litre. The temperature is maintained during 45 minutes at 85° C. and then during a few minutes at 95° C.

One develops in a boiling bath containing 2 g. of sulphuric acid per litre.

According to the dyestuff, one obtains the following hues:

| Coupling product of the diazo-4-phenyl-N-amino-1-benzene-N-sulphonic acid with— | Hue               |                  |
|---------------------------------------------------------------------------------|-------------------|------------------|
|                                                                                 | before developing | after developing |
| (hydroxy-2'-naphthoyl-3')-aminobenzene.....                                     | garnet-red.....   | blue violet.     |
| (hydroxy-2'-naphthoyl-3')-amino-1-methoxy-2-benzene.....                        | do.....           | violet.          |
| (hydroxy-2'-naphthoyl-3')-amino-1-methyl-2-benzene.....                         | do.....           | blue violet.     |

| Coupling product of the methyl-4'-phenyl-N-amino-4-diazo-1-benzene-N-sulphonic acid with— | Hue               |                  |
|-------------------------------------------------------------------------------------------|-------------------|------------------|
|                                                                                           | before developing | after developing |
| (hydroxy-2'-naphthoyl-3')-aminobenzene.....                                               | red violet.....   | reddish blue.    |
| (hydroxy-2'-naphthoyl-3')-amino-1-methyl-2-benzene.....                                   | do.....           | Do.              |

By operating in the same manner with other dyestuffs one obtains the hereafter indicated hues:

| Coupling product of diazo-4-methyl-N-amino-1-benzene-N-sulphonic acid with— | Hue               |                         |
|-----------------------------------------------------------------------------|-------------------|-------------------------|
|                                                                             | before developing | after developing        |
| (hydroxy-2'-naphthoyl-3')-aminobenzene.....                                 | garnet-red.....   | violet-blue.            |
| (hydroxy-2'-naphthoyl-3')-amino-1-methyl-2-benzene.....                     | bordeaux-red..... | Do.                     |
| (hydroxy-2'-naphthoyl-3')-amino-1-methyl-2-methoxy-4-benzene.....           | do.....           | purplish-blue.          |
| (hydroxy-2'-naphthoyl-3')-amino-1-methoxy-2-benzene.....                    | do.....           | violet.                 |
| (hydroxy-2'-naphthoyl-3')-amino-2-benzene.....                              | garnet-red.....   | purplish-blue.          |
| (hydroxy-2'-naphthoyl-3')-amino-1-methoxy-2-benzene.....                    | do.....           | violet-blue.            |
| (hydroxy-2'-naphthoyl-3')-amino-1-methyl-2-methoxy-4-benzene.....           | do.....           | slightly purplish-blue. |
| (hydroxy-2'-naphthoyl-3')-amino-1-methyl-2-benzene.....                     | do.....           | Do.                     |
| (hydroxy-2'-naphthoyl-3')-amino-2-naphthalene.....                          | do.....           | purplish-blue.          |
| (hydroxy-2'-naphthoyl-3')-amino-1-methoxy-4-benzene.....                    | reddish grey..... | grey-green.             |

| Coupling product of the di-methyl-1-N-amino-2-diazo-4-benzene-N-sulphonic acid with— | Hue                  |                  |
|--------------------------------------------------------------------------------------|----------------------|------------------|
|                                                                                      | before developing    | after developing |
| phenyl-methyl-pyrazolone.....                                                        | yellow.....          | salmon-pink.     |
| hydroxy-2-naphthalene.....                                                           | orange-coloured..... | Do.              |
| (hydroxy-2'-naphthoyl-3')-aminobenzene.....                                          | scarlet-red.....     | brownish garnet. |
| (hydroxy-2'-naphthoyl-3')-amino-1-ethoxy-2-benzene.....                              | do.....              | red brown.       |
| (hydroxy-2'-naphthocarbazol-carboxyl-3')-amino-1-methoxy-4-benzene.....              | violet brown.....    | violet brown.    |
| (hydroxy-2'-carbazol-carboxyl-3')-amino-1-chloro-4-benzene.....                      | brownish yellow..... | brown.           |
| terephthaloyl-di(acetyl amino)-1-dimethoxy-2,4-chloro-5-benzene.....                 | yellow.....          | orange brown.    |

| Coupling product of the methyl-4'-phenyl-N-amino-4-diazo-1-benzene-N-sulphonic acid with— | Hue                     |                         |
|-------------------------------------------------------------------------------------------|-------------------------|-------------------------|
|                                                                                           | before developing       | after developing        |
| (hydroxy-2'-naphthoyl-3')-aminobenzene.....                                               | steely blue garnet..... | slightly reddish blue.  |
| (hydroxy-2'-naphthoyl-3')-amino-1-methyl-2-benzene.....                                   | do.....                 | Do.                     |
| phenyl-methyl-pyrazolone.....                                                             | yellow orange.....      | brownish red.           |
| $\beta$ -naphthol.....                                                                    | scarlet red.....        | purplish brown.         |
| (hydroxy-2'-naphthoyl-3')-aminobenzene.....                                               | red violet.....         | bright blue.            |
| (hydroxy-2'-naphthoyl-3')-amino-1-methoxy-4-benzene.....                                  | garnet-red.....         | slightly reddish blue.  |
| (hydroxy-2'-naphthoyl-3')-amino-1-methoxy-2-benzene.....                                  | red brown.....          | Do.                     |
| (hydroxy-2'-naphthoyl-3')-amino-1-ethoxy-2-benzene.....                                   | garnet-red.....         | purplish-blue.          |
| (hydroxy-2'-naphthoyl-3')-amino-1-methyl-2-benzene.....                                   | do.....                 | slightly greenish blue. |
| (hydroxy-2'-naphthoyl-3')-amino-1-nitro-3-benzene.....                                    | violet.....             | blue.                   |
| (hydroxy-2'-naphthoyl-3')-amino-1-methyl-2-methoxy-4-benzene.....                         | garnet-red.....         | slightly reddish blue.  |
| (hydroxy-2'-naphthoyl-3')-amino-1-dimethoxy-2,5-benzene.....                              | do.....                 | purplish blue.          |
| (hydroxy-2'-naphthoyl-3')-amino-1-methyl-2-benzene.....                                   | blue violet.....        | green.                  |
| di(acetyl acetamino)-4,4'-dimethyl-3,3'-diphenyl.....                                     | yellow.....             | brownish yellow.        |
| (hydroxy-2'-carbazol-carboxyl-3')-amino-1-chloro-4-benzene.....                           | brown.....              | violet.                 |
| (hydroxy-3'-diphenylene oxide-carboxyl-2')-amino-1-dimethoxy-2,5-benzene.....             | brown yellow.....       | brownish garnet.        |
| di(hydroxy-2'-naphthoyl-3'-amino)4,4'-dimethoxy-3,3'-diphenyl.....                        | garnet-red.....         | grey blue.              |

Coupling product of the methoxy-4'-phenyl-N-amino-4-diazo-1-benzene-N-sulphonic acid with—

(hydroxy-2'-naphthoyl-3')-aminobenzene.....  
 (hydroxy-2'-naphthoyl-3')-amino-1-methyl-2-benzene.....  
 (hydroxy-2'-naphthoyl-3')-amino-1-methoxy-2-benzene.....  
 (hydroxy-2'-naphthoyl-3')-amino-1-methoxy-4-benzene.....  
 (hydroxy-2'-naphthoyl-3')-amino-1-methyl-2-methoxy-4-benzene.....  
 (hydroxy-2'-naphthoyl-3')-amino-1-dimethoxy-2,5-benzene.....  
 di-(acetylacetamino)-4,4'-dimethyl-3,3'-diphenyl.....  
 (hydroxy-2'-carbazolcarbonyl-3')-amino-1-chloro-4-benzene.....  
 (hydroxy-3'-diphenylene oxide carbonyl-2')-amino-dimethoxy-2,5-benzene.....  
 phenyl-methyl-pyrazolone.....  
 $\beta$  naphthol.....

| Hue                  |                        |
|----------------------|------------------------|
| before developing    | after developing       |
| red violet           | blue.                  |
| do                   | Do.                    |
| do                   | slightly reddish blue. |
| do                   | Do.                    |
| reddish blue.        | Do.                    |
| Do.                  | reddish yellow.        |
| reddish yellow.      | dull violet.           |
| dull orange-coloured | dull purplish red.     |
| red                  | red.                   |
|                      | bordeaux red.          |

Coupling product of the diazo-4-methyl-N-amino-1-benzene-N-sulphonic acid with—

(hydroxy-2'-naphthoyl-3')-amino-1-methoxy-2-benzene.....  
 (hydroxy-2'-naphthoyl-3')-aminobenzene.....  
 (hydroxy-2'-naphthoyl-3')-amino-1-methyl-2-benzene.....  
 (hydroxy-2'-naphthoyl-3')-amino-1-methyl-2-methoxy-4-benzene.....

| Hue               |                  |
|-------------------|------------------|
| before developing | after developing |
| red               | dull violet.     |
| do                | Do.              |
| do                | Do.              |
| do                | Do.              |

Coupling product of the dimethyl-1-N-amino-2-diazo-4-benzene-N-sulphonic acid

(hydroxy-2'-naphthoyl-3')-amino-1-ethoxy-2-benzene.....  
 (hydroxy-2'-naphthoyl-3')-aminobenzene.....  
 (hydroxy-2'-naphthocarbazol-carbonyl-3')-amino-1-methoxy-4-benzene.....  
 (hydroxy-2'-carbazol-carbonyl-3')-amino-1-chloro-4-benzene.....  
 (hydroxy-2'-naphthoyl-3')-amino-1-methyl-2-methoxy-4-benzene.....  
 terephthaloyl-di (acetylamino)-1-dimethoxy-2,4-chloro-5-benzene.....  
 phenyl-methyl-pyrazolone.....  
 naphthol-2.....

| Hue                   |                          |
|-----------------------|--------------------------|
| before developing     | after developing         |
| red                   | dull violet.             |
| do                    | dull red violet.         |
| dark red              | black violet.            |
| violet                |                          |
| yellow brown          | brown.                   |
| red                   | dull violet.             |
| yellow                | slightly reddish yellow. |
| yellow-orange colored | reddish yellow.          |
| red                   | dull red.                |

The hue obtained is identical if the developing is effected in the exhausted dyeing bath to which the necessary sulphuric acid is added in order to obtain a slight blue coloration on Congo red indicating paper.

#### Example 3

1 part of non-loaded silk is dyed on boiling in 30 parts of water containing 0.08 part of borax and 0.2 part of the dyestuff obtained by coupling methoxy-4'-phenyl-N-amino-4-diazobenzene-N-sulphonic acid with (hydroxy-2'-naphthoyl-3')-amino-1-methyl-2-benzene, said coupling being effected following the indications given in Example 2 of the above mentioned co-pending application. One develops as in Example 2; before developing, the hue is red-violet; it turns blue after developing.

In order to avoid the use of a special developing bath it is possible to develop the hue in the very dyeing bath by adding to the latter, after exhaustion, a sufficient quantity of acid in order that it turns the Congo red paper blue. One operates as indicated above: the hues obtained are identical.

#### Example 4

A colour is prepared with the following composition:

|                                          |       |
|------------------------------------------|-------|
| Dyestuff                                 | 40    |
| Thiodiglycol                             | 120   |
| Acetine                                  | 30    |
| Urea                                     | 50    |
| 45 Water and starch-tragacanth thickener | 760   |
|                                          | 1,000 |

One prints on a cotton fabric, dries and passes 50 during one minute through a boiling bath containing 9 g. of sulphuric acid and 100 g. of sodium sulphate per litre. One washes and soaps during half an hour in a bath containing 3 g. of soap and 5 g. of sodium carbonate per litre. This 55 operation is effected while boiling except for the last six dyestuffs of the following list, for which the operation is effected at 80° C. By using the various dyestuffs quoted hereafter and prepared according to the indications of the above mentioned co-pending application one obtains printings which are generally very fast with the hereafter indicated hues. The hues before developing have also been mentioned.

Coupling product of the methoxy-4'-phenyl-N-amino-4-diazobenzene-N-sulphonic acid with—

(hydroxy-2'-naphthoyl-3')-amino-1-methyl-2-methoxy-4-benzene.....  
 (hydroxy-2'-naphthoyl-3')-amino-1-benzene.....  
 (hydroxy-2'-naphthoyl-3')-amino-1-methoxy-2-benzene.....  
 di-(acetylacetamino)-4,4'-methyl-3,3'-diphenyl.....  
 (hydroxy-2'-naphthoyl-3')-amino-1-methyl-2-benzene.....  
 (hydroxy-2'-carbazolcarbonyl-3')-amino-1-chloro-4-benzene.....  
 (hydroxy-2'-naphthoyl-3')-amino-1-methoxy-4-benzene.....  
 $\beta$  naphthol.....  
 phenyl-methyl-pyrazolone.....

| Hue               |                  |
|-------------------|------------------|
| before developing | after developing |
| dull violet       | blue.            |
| garnet red        | Do.              |
| yellow            | reddish blue.    |
| brown             | yellow brown.    |
| do                | blue.            |
| violet            | dull violet.     |
| red               | blue.            |
| yellow brown      | brown.           |
|                   | red.             |

| Coupling product of the phenylamino-4-diazo-benzene-N-sulphonic acid with— | Hue               |                  |
|----------------------------------------------------------------------------|-------------------|------------------|
|                                                                            | before developing | after developing |
| (hydroxy-2'-naphthoyl-3')-aminobenzene.....                                | dark violet.....  | reddish blue.    |
| (hydroxy-2'-naphthoyl-3')-amino-1-methoxy-2-benzene.....                   | dark brown.....   | blue-violet.     |
| (hydroxy-2'-naphthoyl-3')-amino-1-methyl-2-methoxy-4-benzene.....          | violet.....       | reddish blue.    |
| (hydroxy-2'-naphthoyl-3')-amino-2-naphthalene.....                         | black brown.....  | Do.              |
| (hydroxy-2'-naphthocarbazol-carboxyl-3')-amino-1-methoxy-4-benzene.....    | do.....           | blue black.      |

| Coupling product of the methyl-4'-phenyl-N-amino-4-diazo-benzene-N-sulphonic acid with— | Hue               |                  |
|-----------------------------------------------------------------------------------------|-------------------|------------------|
|                                                                                         | before developing | after developing |
| (hydroxy-2'-naphthoyl-3')-aminobenzene.....                                             | dark brown.....   | reddish blue.    |
| (hydroxy-2'-naphthoyl-3')-amino-1-methyl-2-benzene.....                                 | do.....           | Do.              |

| Coupling product of the diazo-4-methyl-N-amino-benzene-N-sulphonic acid with— | Hue               |                    |
|-------------------------------------------------------------------------------|-------------------|--------------------|
|                                                                               | before developing | after developing   |
| (hydroxy-2'-naphthoyl-3')-amino-1-methoxy-2-benzene.....                      | red.....          | grey blue.         |
| (hydroxy-2'-naphthoyl-3')-amino-1-methyl-2-benzene.....                       | red brown.....    | brown violet.      |
| (hydroxy-2'-naphthoyl-3')-amino-1-methyl-2-methoxy-4-benzene.....             | brown violet..... | reddish blue.      |
| (hydroxy-2'-naphthoyl-3')-aminobenzene.....                                   | do.....           | reddish grey blue. |
| di(hydroxy-2'-naphthoyl-3'-amino)-4,4'-dimethoxy-3,3'-diphenyl.....           | brown.....        | reddish blue.      |

| Coupling product of the diazo-4-methyl-amino-2-methylbenzene-N-sulphonic acid with— | Hue               |                  |
|-------------------------------------------------------------------------------------|-------------------|------------------|
|                                                                                     | before developing | after developing |
| (hydroxy-2-naphthoyl-3)-aminobenzene.....                                           | scarlet red.....  | brown violet.    |
| (hydroxy-2'-carbazol-carboxyl-3')-amino-benzene.....                                | yellow brown..... | yellow brown.    |
| (hydroxy-2'-naphthoyl-3')-amino-1-ethoxy-2-benzene.....                             | scarlet red.....  | brown violet.    |
| (hydroxy-2'-naphthocarbazol-carboxyl-3')-amino-1-methoxy-4-benzene.....             | dark brown.....   | black.           |
| di(hydroxy-2'-naphthoyl-3'-amino)-4,4'-dimethoxy-3,3'-diphenyl.....                 | brown.....        | brown violet.    |
| terephthaloyl-di(acetylamino)-1-dimethoxy-2,4-chloro-5-benzene.....                 | yellow.....       | orange-coloured. |
| phenyl-methyl-pyrazolone.....                                                       | do.....           | Do.              |
| hydroxy-2-naphthalene.....                                                          | orange red.....   | red violet.      |

By mixing equal parts of the colours obtained with the dyestuffs prepared, on one hand, with methoxy-4'-phenyl-N-amino-4-diazobenzene - N sulphonic acid and (hydroxy-2'-naphthoyl-3')-amino-1-methoxy-2-benzene and, on the other hand, with the same diazoic and di(acetylacet-amino)-4,4'-dimethyl-3,3'-diphenyl one obtains patterns the colour of which verges to black.

#### Example 5

Fabrics printed and dried as in the preceding example are developed during 15 minutes at 100° C. in saturating steam containing acetic acid. The obtained hues are identical with those developed by using the method according to the said example.

#### Example 6

The following colour is prepared with the dyestuff obtained according to Example 2 of the above mentioned co-pending application by coupling methoxy-4'-phenyl-N-amino-4-diazobenzene-N-sulphonic acid with (hydroxy-2'-naphthoyl-3')-amino-1-methyl-2-methoxy-4-benzene:

Dyestuff ..... 40  
Thiodiglycol ..... 150  
10% solution of ammonium sulphocyanide ..... 20  
Water and starch-tragacanth thickener ..... 790

One prints on cotton, dries, steams during 2 minutes in saturating steam at 100° C. One washes, soaps and dries in the usual manner. One obtains blue patterns.

#### Example 7

One introduces into 50 parts of water 1 part of the dyestuff obtained according to Example 2 of the above mentioned co-pending application by coupling the methoxy-4'-phenyl-N-amino-4-diazobenzene-N-sulphonic acid with the (hydroxy-2'-naphthoyl-3')-amino-1-methoxy-2-benzene; one acidulates with sulphuric acid and boils during 5 minutes. One thus obtains an insoluble dyestuff formed of the desulphonated primitive dyestuff.

What I claim is:

1. A method for coloring fibres, which comprises the steps of applying to said fibres a soluble azoic dyestuff of the general formula



wherein A represents a benzenic nucleus, R is a radical selected from the group consisting of the methyl, phenyl and methoxyphenyl radicals, and R' is the remainder of a hydroxylated coupling component free from any solubilizing group and which is bound to the azo group in a position adjacent to the hydroxyl group, and thereafter

subjecting said soluble dyestuff thus applied to said fibres to an acid treatment, whereby said soluble dyestuff is transformed into an insoluble dyestuff.

2. A method for dyeing animal fibres which comprises the steps of applying to said animal fibres a soluble azoic dyestuff of the general formula



wherein A represents a benzenic nucleus, R is a radical selected from the group consisting of the methyl, phenyl and methoxyphenyl radicals, and R' is the remainder of a hydroxylated coupling component free from any solubilizing group and which is bound to the azo group in a position adjacent to the hydroxyl group, and thereafter subjecting said soluble dyestuff thus applied to said fibres to an acid treatment, whereby said soluble dyestuff is transformed into an insoluble dyestuff.

3. A method for printing cellulosic fibres which comprises the steps of applying to said cellulosic fibres a soluble azoic dyestuff of the general formula



wherein A represents a benzenic nucleus, R is a radical selected from the group consisting of the methyl, phenyl and methoxyphenyl radicals, and R' is the remainder of a hydroxylated coupling component free from any solubilizing group and which is bound to the azo group in a position adjacent to the hydroxyl group, and thereafter treating said soluble dyestuff thus applied to said cellulosic fibres in an acid bath, whereby said soluble dyestuff is transformed into an insoluble dyestuff.

4. A method for printing cotton fibres which comprises the steps of applying to said cotton fibres a soluble azoic dyestuff of the general formula



wherein A represents a benzenic nucleus, R is a radical selected from the group consisting of the methyl, phenyl and methoxyphenyl radicals, and R' is the remainder of a hydroxylated coupling component free from any solubilizing group and which is bound to the azo group in a position adjacent to the hydroxyl group, and thereafter treating said soluble dyestuff thus applied to said cotton fibres in an acid bath, whereby said soluble dyestuff is transformed into an insoluble dyestuff.

5. A method for printing cellulosic fibres which comprises the steps of applying to said cellulosic fibres a soluble azoic dyestuff of the general formula



wherein A represents a benzenic nucleus, R is a radical selected from the group consisting of the methyl, phenyl and methoxyphenyl radicals, and R' is the remainder of a hydroxylated coupling component free from any solubilizing group and which is bound to the azo group in a position adjacent to the hydroxyl group, and thereafter steam treating said soluble dyestuff thus applied to said cellulosic fibres in the presence of an ammonium salt, whereby said soluble dyestuff is transformed into an insoluble dyestuff.

15 6. A method for printing cotton fibres which comprises the steps of applying to said cotton fibres a soluble azoic dyestuff of the general formula



wherein A represents a benzenic nucleus, R is a radical selected from the group consisting of the methyl, phenyl and methoxyphenyl radicals, and R' is the remainder of a hydroxylated coupling component free from any solubilizing group and which is bound to the azo group in a position adjacent to the hydroxyl group, and thereafter 25 steam treating said soluble dyestuff thus applied to said cotton fibres in the presence of an ammonium salt, whereby said soluble dyestuff is transformed into an insoluble dyestuff.

ROBERT LAZARE LANTZ.

#### REFERENCES CITED

The following references are of record in the 45 file of this patent:

#### UNITED STATES PATENTS

| Number    | Name               | Date          |
|-----------|--------------------|---------------|
| 1,362,936 | Fritzsche          | Dec. 21, 1920 |
| 1,483,798 | Green et al.       | Feb. 12, 1924 |
| 1,536,713 | Heusner et al.     | May 5, 1925   |
| 1,745,676 | Hoffa et al.       | Feb. 4, 1930  |
| 1,750,057 | Schirmacher et al. | Mar. 11, 1930 |
| 1,795,125 | Heusner et al.     | Mar. 3, 1931  |
| 2,080,043 | Heckert            | May 11, 1937  |
| 2,172,307 | Gaspar             | Sept. 5, 1939 |
| 2,172,308 | Gaspar             | Sept. 5, 1939 |
| 2,241,247 | Dickey             | May 6, 1941   |

#### FOREIGN PATENTS

| Number  | Country       | Date         |
|---------|---------------|--------------|
| 389,758 | Great Britain | Mar. 23 1933 |